

# UNITED STATES PATENT OFFICE.

CHARLES N. WAITE AND JOSEF E. HEDIN, OF WILMINGTON, DELAWARE, ASSIGNEES OF  
ONE-THIRD TO WILLIAM H. SHARP, OF PHILADELPHIA, PENNSYLVANIA.

## MANUFACTURE OF CHEMICAL SULFATE PULP.

1,249,287.

Specification of Letters Patent.

Patented Dec. 4, 1917.

No Drawing.

Application filed February 8, 1914. Serial No. 816,168.

*To all whom it may concern:*

Be it known that we, CHARLES N. WAITE and JOSEF E. HEDIN, of the city of Wilmington, county of Newcastle, and State of Delaware, have invented certain new and useful Improvements in the Manufacture of Chemical Sulfate Pulp, whereof the following is a specification.

Our invention relates to improvements in the art of manufacturing chemical sulfate pulp as used in paper manufacture, and more particularly to the solution which is used in such processes for the purpose of cooking or digesting the wood. Sodium sulfid has heretofore been used in solution for this purpose, but it has been customary to obtain the sodium sulfid by the smelting of sulfate of soda with a mixture of carbonate of soda and organic matter contained in the black liquor as the result of a preceding process of digestion.

According to our process, we obtain the sulfid of sodium in the digesting liquor by the direct addition of sulfur to a caustic soda solution.

In the practice of our process we add to a solution of caustic soda (say about seven per cent. or eleven degrees Baumé) a sufficient amount of sulfur to produce a suitable quantity of sodium sulfid by reaction with the caustic soda. For ordinary purposes, we find that the addition of sulfur in the amount of about two per cent. of the total liquor used produces good results. The sulfur should be added to the caustic soda solution while boiling, and the process should be continued for about three hours before the liquor is ready for use.

As the result of the addition of the sulfur a portion of the caustic soda has been converted into sodium sulfid leaving additional caustic soda not affected. The liquor thus formed is added in the usual digester to the wood and the process of digesting practised as known to those skilled in this art.

In this process the liquor digests the wood with formation of a waste black liquor which is drawn off from the wood pulp which is to be used in paper manufacture. Thereafter the waste liquor is returned and from it carbonate of soda is recovered by the usual process which consists in evaporating the water and burning out the organic matter which leaves carbonate of soda. This carbonate of soda is then dissolved and lime

added for the production of caustic soda. According to our process it is convenient to add the sulfur required along with the lime during this causticizing process, thereby avoiding the necessity of a separate process for the production of the sodium sulfid.

After having thus added the sulfur during the causticizing process with the production of sodium sulfid, the liquor is then again used and the process repeats itself.

By our process the formation of the digesting liquor is much simplified. The use of any smelting process is avoided and the proportion of sodium sulfid in the liquor may be regulated with much greater nicety than in previous processes.

There is a corresponding saving of the cost of raw material.

Having thus described our invention, we claim:

1. The process of manufacturing liquor to be used in the digestion of wood pulp, which consists in taking the spent liquor remaining from a previous digestion, evaporating the water therefrom, burning out the organic matter contained, dissolving the resulting sodium carbonate and at the same time adding lime, whereby caustic soda is produced, and sufficient sulfur to convert part of the caustic soda into sodium sulfid, and using the liquor thus produced for a succeeding process of digesting wood.

2. The process of digesting wood pulp for the manufacture of paper, which consists in adding to a caustic soda solution a quantity of sulfur sufficient to convert a portion of the caustic soda into sodium sulfid, and thereafter adding the liquor thus produced to the wood to be digested, drawing off from the digested wood pulp the resulting liquor, evaporating the water therefrom, burning the organic matter, dissolving the remaining carbonate of soda and adding thereto lime and sulfur whereby there is produced a solution containing caustic soda and sodium sulfid and using the liquor thus produced for a succeeding process of digesting wood.

In testimony whereof, we have hereunto signed our names at Philadelphia, Pennsylvania, this thirty-first day of January, 1914.

CHARLES N. WAITE.

JOSEF E. HEDIN.

Witnesses:

JAMES H. BELL,  
E. L. FULLERTON.